

## UNITED STATES PATENT OFFICE

2,475,134

## SULFITE ANTISTAIN BATH FOR MULTI-LAYER COLOR FILM

Harold C. Harsh and James E. Bates, Binghamton, N. Y., assignors to General Aniline & Film Corporation, New York, N. Y., a corporation of Delaware

No Drawing. Application November 8, 1945,  
Serial No. 627,533

9 Claims. (Cl. 95—2)

1

This invention relates to photographic anti-stain baths, to anti-stain baths employed in multi-color photography, and especially to non-staining baths for the washing of multi-color photographic material following the fixing treatment.

It is known that in the processing of multi-color reversible film and multi-color reversible film coated upon a white opaque support, the exposed film or exposed white opaque, is first developed with a normal black and white developer to produce a negative image. After development, the black and white negative material, without being fixed, is exposed to general illumination, followed by a second development with a color-forming developer. During the first and second development the silver-halides in all the layers are reduced to metallic silver. After the second development, the material is cleared in running water, hardened in an aqueous solution consisting of either chrome or potassium alum, and then washed in running water. After the latter treatment, the silver present in all the layers formed during the first and second development is converted into a salt by any of the known silver-salt formers, commonly known as bleaching baths, and the silver-salt thus formed is then removed by dissolving it in a silver-salt solvent such as, for example, hypo. The material is then washed for a long period of time and then dried.

Prior to the washing operation it is essential that the residual second or color developer and bleach solutions be removed, otherwise stains will be formed during the drying operation, which are particularly noticeable in the white area. In order to prevent this staining, an extended final washing time in running water of from fifteen minutes to two hours, has been proposed. Even if this proposal be adopted, stains are nevertheless formed after the drying operation. It is believed that the staining results from the oxidation of traces of the color developer retained in the layers of the material following color-forming development, which then react with the unused color-former.

An object of the present invention is to eliminate excessive washing time of color developer multi-color photographic material while preventing the formation of stain.

A further object of the invention is a final rinse bath which clears undesirable matter from a multi-color photographic material in a short time while avoiding staining.

Other objects and features of the invention will

become more apparent as the description proceeds.

We have found that the above objects are accomplished by employing, as a final rinse bath, an aqueous solution containing a small quantity of a water-soluble alkali sulfite such as ammonium, potassium, or sodium sulfite, bisulfite, and meta-bisulfite. This discovery makes it possible to considerably reduce the final washing time. The concentration of the alkali sulfite may vary from as little as 0.01% to as high as 1%. Amounts higher than 1% give little improvement in stain prevention from a practical standpoint and, accordingly, concentrations ranging from between 0.1% to 1% are most desirable.

The photographic multi-layer materials, which may be processed with the anti-stain bath of the present invention, are color reversible film, color negative film, color reversible printing material 20 coated on a white opaque base, and color positive printing material coated on paper, irrespective of whether the dyestuff images are produced with color-formers present in the emulsion or by a selective second exposure followed by color development. The color reversible film consists of an integral tripack emulsion coated on the usual clear cellulose acetate or nitrate film base. Each of the emulsions are sensitized to one of the primary colors of light; namely, blue, green, and red. The top layer is blue sensitive. A filter layer, yellow in color and blue absorbing, lies under the top layer. Below this filter layer, lies a green sensitive emulsion layer, and below this is a red sensitive emulsion layer. Each of the three 35 silver-halide emulsion layers contain dye-forming compounds which unite during the development of silver image in an aromatic amine developing agent to form a dye with the oxidation product of the developing agent, or may be free from color-formers in which case the film is processed with the color-formers in the color developers by the selective second exposure and color development method as described in United States Patents 1,897,866; 1,900,870; 1,928,709 and 45 1,980,941. The color negative film is made up in the same manner as the color reversible film, with the exception that it may contain a layer of clear gelatin between the red sensitive layer and the green sensitive layer. The color reversible white opaque material is prepared in the same manner as color reversible film and the color negative film, with the exception that the base consists of an opaque white film. The color paper is also constructed in the same manner as the color reversible film and the color negative film, with the ex-

ception that the emulsion is coated on a baryta coated paper base.

As silver is formed during development, it must be removed after color development by treatment in a bleach, followed by treatment in a bath of sodium thiosulfate according to usual practice. A yellow dye is formed in the blue sensitive emulsion; a magenta dye is formed in the green sensitive emulsion; and a cyan dye is formed in the red sensitive emulsion. Combinations of these three printing primaries will produce all of the other colors in the finished film or print. Suitable methods for the preparation of photographic multilayer materials have been described in the literature relating to color photography, and are, therefore, not described here.

The following examples describe in detail methods for accomplishing the above objects, but it is to be understood that they are inserted merely for the purpose of illustration and are not to be construed as limiting the scope of the invention.

*Example I*

A 4" x 5" full color transparency sheet of color film was printed by contact on two 4" x 5" sheets of color reversible white opaque film.

The two sheets of 4" x 5" color reversible white opaque film were first developed for twelve minutes at 68° F. in a developer of the following composition:

|                                     |        |    |
|-------------------------------------|--------|----|
| p-monomethylamine-m-phenol sulphate | grams  | 3  |
| Sodium sulfite                      | do     | 50 |
| Hydroquinone                        | do     | 6  |
| Sodium carbonate (monohydrate)      | do     | 40 |
| Sodium thiocyanate                  | do     | 2  |
| Potassium bromide                   | do     | 2  |
| Water to make up                    | liters | 1  |

The developed film was short stopped for 3 minutes at 68° F., in a 5% aqueous solution of sodium bisulfite.

The film was washed for 2 minutes in running water at 68° F., and then color developed for 15 minutes at 68° F., in a developer of the following composition:

|                           |        |    |
|---------------------------|--------|----|
| p-Aminodiethylaniline HCl | grams  | 4  |
| Sodium sulfite            | do     | 5  |
| Hydroxylamine HCl         | do     | 2  |
| Sodium carbonate          | do     | 40 |
| Potassium bromide         | do     | 1  |
| Water to make up          | liters | 1  |

The color developed film was rinsed for 4 minutes in running water at 68° F., and hardened for 5 minutes in a 3% aqueous solution of potassium chrome alum.

The hardened film was washed for 5 minutes in running water at 68° F. The washed material was then treated with a bleach bath of the following composition:

|                                       |        |     |
|---------------------------------------|--------|-----|
| Di-potassium mono-sodium ferricyanide | grams  | 100 |
| Potassium bromide                     | do     | 15  |
| Disodium phosphate                    | do     | 40  |
| Sodium bisulfate                      | do     | 25  |
| Water to make up                      | liters | 1   |

The bleached film was washed for 5 minutes at 68° F. and then fixed for 5 minutes in a solution of the following composition:

|                  |        |     |
|------------------|--------|-----|
| Hypo             | grams  | 200 |
| Borax            | do     | 10  |
| Water to make up | liters | 1   |

After fixing, the material was washed for 10 minutes in running water at 68° F.

After the final wash, one print was allowed to dry while the other was rinsed for 2 minutes in a 0.1% solution of sodium sulfite and then allowed to dry. At this point the prints appeared identical. After normal drying, the print rinsed in the sodium sulfite solution showed brighter colors and more brilliant highlights than the print given only a water wash for 15-20 minutes.

When the drying was carried out under conditions of high humidity so that the drying time was extended for several hours the water rinsed print showed even greater highlight stains while the print rinsed in sodium sulfite solution did not change.

*Example II*

Example I was repeated with the exception that the colored photographic multilayer material employed was color paper, and the final rinse bath was a 0.01% solution of sodium bisulfite instead of a 0.1% solution of sodium sulfite. The color print washed in water showed objectionable stains after drying, while the print treated with the solution of sodium bisulfite was clear and unstained.

*Example III*

Example I was repeated with the exception that the final rinse bath was a .01% solution of sodium metabisulfite instead of a 0.1% solution of sodium sulfite. After fixing and washing, the color print rinsed in plain water showed objectionable stains, while the print treated with the sodium metabisulfite solution was clear and unstained.

From the above examples it is manifest that the multi-layer photographic material rinsed in plain water shows marked staining upon drying of said material. This staining occurs especially under slow drying conditions and is probably due to the coupling of the slow oxidation product of the color developer with a residual color-coupler present in one or more layers.

In place of the water-soluble alkali sulfite solutions referred to above, a fixing bath consisting of hypo and borax containing an alkali sulfite in quantities ranging from about 3 to 8 grams per liter, may also be employed.

A typical composition of a fixer employing an alkali sulfite is as follows:

|                  |        |     |
|------------------|--------|-----|
| Hypo             | grams  | 200 |
| Borax            | do     | 10  |
| Alkali sulfite   | do     | 3-8 |
| Water to make up | liters | 1   |

The fixing bath as above prepared may be employed in place of the normal fixer and prior to the washing operation after fixing the prints, and given a normal wash of 10 to 20 minutes and allowed to dry.

After drying, the prints will have a clearer highlight than the prints fixed in the usual fixing bath and then washed for 10 to 20 minutes.

The above specific examples are to be regarded as merely illustrative of the invention, and not in any sense restrictive. It will be obvious to anyone skilled in the art that many modifications such as substituting equivalent material and varying the proportions of materials used are within the spirit and scope of the invention as defined in the appended claims.

We claim:

1. In a process of color photography the method of preventing stains on color images selected

from the class consisting of indophenol and azomethine dyes, produced in a multilayer color film by color-forming development which comprises washing said film after exposure, color developing, bleaching and fixing, but prior to drying with an aqueous solution consisting of water and an alkali sulfite.

2. In a process of color photography the method of preventing stains on color images selected from the class consisting of indophenol and azomethine dyes, produced in a multilayer color film by color-forming development which comprises washing said film after exposure, color developing, bleaching and fixing, but prior to drying with an aqueous solution consisting of water and sodium sulfite.

3. In a process of color photography the method of preventing stains on color images selected from the class consisting of indophenol and azomethine dyes, produced in a multilayer color film by color-forming development which comprises washing said film after exposure, color developing, bleaching and fixing, but prior to drying with an aqueous solution consisting of water and sodium bisulfite.

4. In a process of color photography the method of preventing stains on color images selected from the class consisting of indophenol and azomethine dyes, produced in a multilayer color film by color-forming development which comprises washing said film after exposure, color developing, bleaching and fixing, but prior to drying with an aqueous solution consisting of water and sodium metabisulfite.

5. The method according to claim 1 wherein the concentration of the said alkali sulfite ranges from .01% to 1%.

6. In a process of producing color photographic images selected from the class consisting of indophenol and azomethine dyes, in a multilayer color film by exposing the film, color-forming developing the same, bleaching, fixing and washing, the improvement which comprises avoiding the formation of stain, after the bleaching, fixing, and washing operation, by rinsing the said film with an aqueous solution consisting of water and an alkali sulfite.

7. In a process of producing color photographic images selected from the class consisting of indophenol and azomethine dyes, in a multi-

5 layer color film by exposing the film, color-forming developing the same, bleaching, fixing and washing, the improvement which comprises avoiding the formation of stain, after the bleaching, fixing, and washing operations, by rinsing the film with an aqueous solution consisting of water and sodium sulfite.

8. In a process of producing color photographic images selected from the class consisting of indophenol and azomethine dyes, in a multilayer color film by exposing the film, color-forming developing the same, bleaching, fixing and washing, the improvement which comprises avoiding the formation of stain, after the bleaching, fixing, and washing operations, by rinsing the film with an aqueous solution consisting of water and sodium bisulfite.

9. In a process of producing color photographic images selected from the class consisting of indophenol and azomethine dyes, in a multilayer color film by exposing the film, color-forming developing the same, bleaching, fixing and washing, the improvement which comprises avoiding the formation of stain, after the bleaching, fixing, and washing operations, by rinsing the film with an aqueous solution consisting of water and sodium metabisulfite.

HAROLD C. HARSH.  
JAMES E. BATES.

#### REFERENCES CITED

The following references are of record in the file of this patent:

#### UNITED STATES PATENTS

| Number       | Name    | Date           |
|--------------|---------|----------------|
| 1,617,434    | Binder  | Feb. 15, 1927  |
| 1,753,059    | Murray  | Apr. 1, 1930   |
| 1,930,140    | Becker  | Oct. 10, 1933  |
| 40 2,059,884 | Mannes  | Nov. 3, 1936   |
| 2,203,903    | Ham     | June 11, 1940  |
| 2,301,387    | Evans   | Nov. 10, 1942  |
| 2,323,481    | McQueen | July 6, 1943   |
| 2,384,658    | Vittum  | Sept. 11, 1945 |

#### OTHER REFERENCES

Clerc, "Photography Theory and Practice," 2d edition, 1937, published by Sir Isaac Pitman and Sons Ltd., pages 236 and 237 cited.